

## UNITED STATES PATENT OFFICE

2,201,425

## ALLOY STEEL

Karl Torkel Berglund, Sandviken, Sweden, assignor to Sandvikens Jernverks Aktiebolag, Sandviken, Sweden, a company of Sweden

No Drawing. Application April 28, 1938, Serial No. 204,754. In Sweden May 3, 1937

2 Claims. (Cl. 75—125)

The present invention relates to an alloy steel which is capable of being hardened to martensitic structure, and which is particularly adapted to be used for the manufacture of corrosion re-

5 sistant hardened articles, such as pointed tools and tools having a cutting edge.

Corrosion resistant chromium steels that are capable of being hardened to martensitic structure are, generically speaking, built up on an alloy base the composition of which lies within the following approximate limits:

|                        | Per cent  |
|------------------------|-----------|
| Carbon                 | 0.20—2.50 |
| Chromium               | 8—22      |
| 15 Iron, maximum about | 90        |

Having regard to the resistance to corrosion the lower limit of the chromium content of all of these steels may be placed at about 12%. With 20 less exacting requirements as to resistancy to corrosion, somewhat lower chromium contents may also be used. The upper limit of the chromium content is at about 20%, having regard to the hardenability of the steels.

25 The carbon content that is most suitable for different fields of use is determined, in the main, by the maximum hardness that it is sought to attain by hardening, and also by the desired qualities of the edge of the tool. The maximum hardness that it is possible to obtain by hardening, increases with increasing carbon content, but simultaneously, the difficulties connected with shaping and working the steel in hot and cold state also increase.

35 If the steel is to be used for articles having a thin cutting edge of a sufficient durability for practical purposes, a carbon content of at least 0.50%, and preferably not lower than 0.70%, is required. An increased carbon content gives as 40 a rule a better edge, but having regard to the possibility of working the steel by cold rolling and cold drawing and to the difficulties of rendering the carbides in a sufficiently finely divided state, a higher carbon content than about 1.35% can hardly be considered for this purpose. The 45 improved edge obtained through an increased carbon content is explained by the increased quantity of hard and wear-resistant carbides. An increased carbide content, however, impairs as a rule the resistancy to corrosion of the steel, due to the chromium content of the carbides being so high that the chromium content of the ground mass is reduced.

According to existing equilibrium diagrams of 55 the alloy system iron-chromium-carbon, two carbides can exist within the range of concentration here contemplated, namely, a trigonal carbide  $(\text{Cr},\text{Fe})_7\text{C}_3$  and a cubic carbide  $(\text{Cr},\text{Fe})_4\text{C}$  or, probably more correctly,  $(\text{Cr},\text{Fe})_{23}\text{C}_6$ . At temperatures above about  $800^\circ\text{C}$ . only the trigonal car-

bide can exist when equilibrium is attained, whereas at temperatures below about  $800^\circ\text{C}$ . also the cubic carbide appears together with the trigonal one.

5 Generically speaking the conclusion may be drawn that for one and the same carbon content the amount by weight of carbides when in the cubic phase should be 1.5 to 1.8 times the amount obtained if the carbides are in the trigonal phase. On the other hand, owing to its greater quantity 10 the cubic carbide may occasion that, for a certain chromium content of the steel, the ground mass becomes poorer in chromium, with the resultant risk of inferior resistancy to corrosion.

According to the present invention the carbides 15 or at least the greater portion of the same may be obtained in the cubic phase by incorporating with a chromium steel containing 0.20 to 1.35% carbon and 8 to 22% chromium, a further alloy component of molybdenum, cobalt and copper. 20 The steel according to the present invention is thus mainly characterized by that, in addition to an alloy base of the composition above set forth, and normal amounts of manganese, silicon, phosphorus, and sulphur present in commercial iron and steel, it also contains the combined alloy component molybdenum-cobalt-copper, the content of these elements being each at least 0.20% and together at least 0.60% and at the most 15% of the weight of the steel thus alloyed. Molybdenum may be wholly or partially replaced by tungsten.

25 It has been proved by tests that the resistancy to corrosion of an alloy steel according to this invention is not impaired but, on the contrary, is improved both in the annealed state and, above all, in the hardened state.

30 This twofold effect of a combined alloy component of molybdenum, cobalt and copper was not to be expected in view of the fact that a 35 moderate addition of one of these elements alone does not result in any noticeable deviation from the equilibrium diagram for iron-chromium-carbon alone.

35 In addition to the gain of an improved resistancy to corrosion due to the said combined addition of alloy components, the advantage of a larger quantity of carbides for a given carbon content is also gained, and thus greater hardness and increased wearing strength in the hardened state, and it has also been found that the complex cubic carbide that is formed under these conditions, can more easily be obtained in a finely dispersed state in connection with the shaping of the material.

40 Since the chromium carbides are particularly 45 resistant to action of chemicals, they are obtained as an undissolved residue if the annealed steel is dissolved, for instance, in diluted hydrochloric acid. The solution is preferably made in an at-

mosphere of carbon dioxide so as to eliminate the risk of the carbides being oxidized by the oxygen of the air. A great number of tests have given the result that in the case of a chromium 5 steel containing about 1% carbon and from 13 to 14% chromium but having no other intentional alloy components, the quantity of the carbides amount to from 7 to 8 per cent of the weight of the steel.

10 A further addition of moderate quantities of manganese, cobalt or copper does not noticeably change the quantity of the carbides. On the other hand, a certain increase of the quantity of carbides is obtained by an addition of 15 tungsten or molybdenum. If, however, in accordance with the present invention, a composite addition of molybdenum, cobalt and copper is made, for instance, about 1% of each substance, the carbide content of the steel is increased to 20 18 or 19%. This increase of the carbide content is quite surprising in view of the fact that cobalt and copper each by itself does not increase the carbide content.

A roentgenographic examination of carbide residues has given the following results: In a chromium steel of this type without extra alloy components the carbides consisted of approximately equal parts trigonal carbide and cubic carbide, and thus conformed with the requirements of the 25 equilibrium diagram. On the other hand, the carbide residue of a chromium steel to which the composite component molybdenum-cobalt-copper had been added, proved to consist practically completely of cubic carbide, in spite of the fact 30 that the said steel had been heated during a long period of time at about 860° C. that is to say, at a temperature range at which, according to available equilibrium diagrams, the trigonal carbide only should be present.

35 40 The great resistancy to corrosion shown by a steel of the said type containing molybdenum-cobalt-copper will be explained in part, it is believed, by the following analyses shown by the carbide residues:

|                                                           | Percent C | Percent Fe | Percent Cr |
|-----------------------------------------------------------|-----------|------------|------------|
| Carbides of a chromium steel with Mo-Co-Cu-addition       | 5.64      | 40.7       | 47.3       |
| Carbides of a chromium steel without extra alloy elements | 8.20      | 26.5       | 63.4       |

The considerably higher iron content and the 55 lower chromium content of the carbides of the complex steel alloyed in accordance with the present invention should result in a smaller electrolytic potential difference between carbide and ground mass than in the simple chromium steel. 60 In this case the original steel showed the following analysis:

|            | Per cent |
|------------|----------|
| Carbon     | 1.02     |
| Manganese  | 0.41     |
| Silicon    | 0.19     |
| Chromium   | 12.9     |
| Molybdenum | 0.95     |
| Cobalt     | 1.49     |
| Copper     | 1.00     |

70 The analysis of the carbide residue of this steel corresponds to the formula



a value which, having regard to the possible

accuracy of analysis, corresponds exceedingly well to the theoretical formula  $(Cr, Fe)_{23}C_6$ , and which is also in keeping with the results of the roentgenographic examination.

It may be pointed out that the addition of copper appears to be of essential importance to the marked increase in resistancy to corrosion as well as to the formation of the desired cubic carbide.

As regards the manganese content it may be mentioned that in a steel according to the present invention the manganese content should be less than 0.65%, since with the composite alloy component here contemplated a greater optimum hardness can be obtained below this limit than at a higher manganese content.

An alloy steel according to the present invention which is particularly suitable for the manufacture of fine hardened edge tools, such as razor blades and surgical instruments, contains:

|            |            |    |
|------------|------------|----|
| Carbon     | 0.70- 1.40 | 20 |
| Chromium   | 10 -18     |    |
| Molybdenum | 0.20- 2    |    |
| Cobalt     | 0.20- 2    |    |
| Copper     | 0.20- 2    | 25 |

For special fields of use it may be desirable slightly to modify the mechanical and other properties of the alloy steels by an addition of further alloy elements, over and above the composite alloy component molybdenum-cobalt-copper. 30 Thus, the steel according to the present invention may contain percentages exceeding 0.05% of one or more of the alloy elements: Beryllium, boron, aluminium, titanium, vanadium, arsenic, selenium, zirconium, niobium, tin, antimony, tantalum, uranium.

Since, as previously stated, molybdenum may be replaced wholly or partially by tungsten, the term "molybdenum" in the following claims should be construed as covering tungsten also.

I claim:

1. An alloy steel of the martensitic type, which is stainless in the hardened condition, characterized by containing when in hardened condition substantially all of the carbides in the cubic phase 45 and possessing great hardness and wearing strength, comprising as its principal alloying ingredients carbon in the proportion of 0.20 to 1.35%, chromium in the proportion of 10 to 22%, nickel less than 0.20%, phosphorus less than 0.05%, molybdenum in the proportion of 0.20 to 5%, cobalt in the proportion of 0.20 to 5%, copper in the proportion of 0.20 to 5%, the remainder being iron with impurities in an amount which will not alter the properties of the alloy.

2. An alloy steel of the martensitic type, which is stainless in the hardened condition, characterized by containing when in hardened condition substantially all of the carbides in the cubic phase 60 and possessing great hardness and wearing strength, comprising as its principal alloying ingredients carbon in the proportion of 0.70 to 1.35%, chromium in the proportion of 10 to 18%, nickel less than 0.20%, phosphorus less than 0.05%, molybdenum in the proportion of 0.20 to 65

2%, cobalt in the proportion of 0.20 to 2%, copper in the proportion of 0.20 to 2%, the remainder being iron with impurities in an amount which will not alter the properties of the alloy.

55

60

65

70

KARL TORKEL BERGLUND.